

Sept. 6, 1938.

F. BLUEN ET AL

2,129,460

LIMESTONE SLAB AND METHOD OF COLORING SAME

Filed Feb. 5, 1937

Fig. 1.



Fig. 2.



12 13 Fig. 3.



Inventors:

Frederick Bluem  
Kurt Bluem

by Davis, Lindsay, Smith & Shantz  
Attn: [unclear]

## UNITED STATES PATENT OFFICE

2,129,460

LIMESTONE SLAB AND METHOD OF COLOR-  
ING SAME

Frederick Bluem and Kurt Bluem, Chicago, Ill.

Application February 5, 1937, Serial No. 124,178

11 Claims. (Cl. 91—68)

Our invention relates generally to the coloring and polishing of ordinary limestone, as distinguished from the so-called marbles, for the purpose of improving its artistic appearance and enlarging its availability for harmonious decorative treatment.

While the color of limestone varies with the amount and character of its oxide content, such as iron oxide, copper oxide, etc., its color value and artistic appeal are considerably below those of the more expensive and decorative stones, such as marble and granite, which, therefore, are particularly adapted for the decorative treatment of interiors. Moreover, the majority of limestones are incapable of taking a marble-like polish, so that where used as the predominating stone in decorating schemes, the result is apt to be drab, cold and lustreless.

It is, therefore, the principal object of our invention to provide a method of coloring limestone to produce any desired colored effect or design and of further conditioning and treating the stone to produce a high polish on the colored surface.

A further object is to provide a polished limestone slab having portrayed thereon any desired color scheme or design which leaves visible the natural texture of the stone, the slab being thoroughly dried and having a protective coating for preventing the subsequent absorption of moisture.

These and further objects of our invention will be set forth in the following specification, reference being had to the accompanying drawing and the novel means by which said objects are effectuated will be definitely pointed out in the claims.

In the drawing:

Figure 1 is a perspective view of a plain, limestone slab before being treated according to our improved method;

Fig. 2 is a plan view of the same slab colored and decorated according to a selected design;

Fig. 3 is an enlarged section along the line 3—3 in Fig. 2, looking in the direction of the arrows and showing the relation of the successive treatments to the stone surface.

In carrying out our improved method, the limestone is first cut into slab-like form and preferably to a thickness varying from  $\frac{1}{2}$ " to 3". At this stage, the surfaces of the slab have the characteristic limestone appearance, as represented generically and in greatly exaggerated form by the numeral 10 in Fig. 3. These relatively thin slabs are employed because of the necessity of preliminarily expelling all contained moisture from the slabs which otherwise might later re-

sult in a peeling or disintegration of the colored surface.

Accordingly, the slabs are heated at a temperature of from 120° to 180° F. for a time sufficient to insure the removal of all contained moisture, the time of heating varying with the thickness of the slab. This heating of the slabs is insufficient to effect any disintegration of the limestone and this step of the treatment is characterized by the further advantage of opening the pores of the stone, thus insuring a firm interlock with the slab of the materials thereafter applied.

The next step in the method consists in applying the colors to the surface of the dried stone. These colors may be applied while the stone is cool, or the stone may be slightly warm, but in any case, it will be understood that, after being dried, the slabs have been so handled as to prevent the reabsorption of moisture.

Since one of the important features of our invention is the preservation of the natural texture of the limestone, regardless of the nature of the coloring or decorative design applied, we prefer to use our colors in the form of stains, rather than in paint form which would otherwise conceal the stone texture. Further, we prefer to use stains of animal or vegetable origin, and, as vehicles therefor, an easily evaporable liquid, such as alcohol, rather than an oily vehicle which is difficult to control when applied to a porous stone, such as limestone. These stains may be prepared in any of the well known ways and their strength may be varied as desired to obtain any color intensity and liquidity of stain.

Any of the stains may be applied by a brush, if the design is of the general nature as illustrated in Fig. 2, but if the complete surface of the slab is to be colored by a single stain, the latter may be applied by spraying. Owing to the nature of the stains employed and the porosity of the stone, a slight surface impregnation of the surface is effected, as indicated by the numeral 11, and, further, due to the lack of hiding power of the stains, the full texture of the stone surface remains visible after coloring, so that the slab retains its stone appearance. Depending upon the original color and surface characteristics of the limestone used, it may be necessary to make more than one application of the desired stains to the surface in order to secure the required depth and tone of color.

After the stains have been applied and the surface of the stone is completely dry, we next apply a simple solution of alcohol and clear white shellac to the colored surface in order to

fill the deeper portions of the stone pores and also provide an extremely thin, bonding layer 12 with the plastic mass or cement 13 that is next applied. This cement comprises equal parts by 5 volume of powdered limestone, clear white, liquid shellac, and the stain originally used for coloring the stone. It will be understood that, if the surface of the slab is originally stained with a single color, then only one similarly colored cement is required but if a decorative design comprising numerous colors is portrayed on the surface, then it is necessary to employ for each colored area a cement that is similarly colored. This cement is characterized generally by the 10 consistency of butter and, due to the presence of the shellac, it is able to form a bonding union with the shellac coating previously applied and so insure the firm holding of the cement in place. This action is facilitated to some extent by the 15 interlocking of the mass with the pores and interstices of the stone surface, the cement acting substantially as a filler in order to facilitate the obtaining of a smooth slab surface that is capable of being polished. This cementitious filler 20 is then permitted to dry which requires from one to three hours. The stone surface is then rubbed down with emery cloth until it is finger smooth and the color and structure of the stone are clearly visible.

30 Thereafter, the conditioned surface is rubbed with a clean white, linen cloth that is dipped in hot olive oil and this oil treatment imparts a slightly glistening appearance to the colored surface. This appearance is preferably enhanced 35 and the surface protected against normal temperature changes by applying a coat 14 of a good commercial grade of waterproof varnish. After the varnish is dry, it is rubbed down with a piece of felt dipped first in vinegar and then 40 in powdered hartshorn. This rubbing serves to reduce the thickness of the varnish coat and to remove brush marks and similar light reflecting disturbances on the surface, so that the surface of the slab is not only glass smooth and polished, 45 but retains the original stone texture. If a duller finish is desired, the varnish coat may be omitted.

The foregoing treatment colors and decorates the surface of the slab so treated, and also renders the treated surface resistant to moisture absorption both with and without the varnish 50 coat, since the presence of the shellac in the cement covering renders the same waterproof. However, in order to protect the slab against moisture absorption through other surfaces, we prefer to coat the untreated surfaces with a solution comprising one and one-half ounces of paraffin which is melted by boiling in one quart of linseed oil. This solution is applied with a brush to the untreated stone surfaces, such as 55 the edge and back surfaces, and it provides a moisture-proof coating 15.

By the use of our improved method, therefore, 60 architects and decorators may harmoniously include ordinary limestone in any desired decorative scheme. The application of the method is not restricted in any substantial way, since it is not only possible to color entire stone surfaces with a single color, but also to incorporate thereon rather complicated designs, such as replicas 65 of the more expensive types of marbles, geometrical and artistic designs of various kinds, and human and animal figures and portraits. One typical arrangement is shown in Fig. 2 which illustrates a vein-like design. Any of these 70 designs may be embodied on a limestone surface

without destroying the stone-appearance of the slab which is a very important advantage, particularly in interior decoration.

We claim:

1. The method of coloring a limestone slab 5 consisting in thoroughly drying the slab, staining the slab surface to be exposed with a selected color, bonding to the stained surface a plastic, cementitious powdered limestone composition having substantially the same color as the original stain, permitting the composition to dry, applying waterproof varnish to the composition treated surface to smooth the same and provide a glistening surface, and then coating the remaining surfaces of the slab with a solution of 10 paraffin to prevent the ingress of moisture.

2. The method of coloring a limestone slab 20 consisting in thoroughly drying the slab, staining the slab surface to be exposed with a selected color, applying clear liquid shellac to the colored surface to fill the deeper pores thereof, covering the shellacked surface with a filler composition comprising limestone dust, white liquid shellac and the stain employed in the original coloring, 25 permitting the composition to dry, applying waterproof varnish to the composition treated surface to smooth the same and provide a glistening surface, and then coating the remaining surfaces of the slab with a solution of paraffin to prevent the ingress of moisture.

3. The method of coloring a limestone slab 30 consisting in thoroughly drying the slab, staining the slab surface to be exposed with a selected color, applying clear liquid shellac to the colored surface to fill the deeper pores thereof, covering 35 the shellacked surface with a filler composition comprising limestone dust, white liquid shellac and the stain employed in the original coloring, permitting the composition to dry, rubbing the surface until finger smooth, applying waterproof 40 varnish to the composition treated surface to further smooth the same and provide a glistening surface, and then coating the remaining surfaces of the slab with a solution of paraffin to prevent 45 moisture absorption.

4. The method of coloring a limestone slab 50 consisting in thoroughly drying the slab, staining the slab surface to be exposed with a selected color, applying clear liquid shellac to the colored surface to fill the deeper pores thereof, covering 55 the shellacked surface with a cementitious filler composition including limestone dust and the stain employed in the original coloring, permitting the composition to dry, rubbing the surface until finger smooth, applying waterproof varnish to the composition treated surface to further 60 smooth the same and provide a glistening surface, rubbing the varnish coat to remove brush marks and provide a substantially polished surface, and then coating the remaining surfaces of the slab with a solution of paraffin to prevent 65 moisture absorption.

5. A limestone slab having a surface stained with a selected color and bonded thereto a thin 70 filler covering in the form of a composition having substantially the same color as the original stain and including powdered limestone, the covered surface being smooth and having the texture of the original slab.

6. A limestone slab having a surface stained with a selected color and bonded thereto a thin 75 filler covering in the form of a composition having substantially the same color as the original stain and including powdered limestone, the covered surface being varnished to present a 80

polished appearance and having the texture of the original slab.

7. A limestone slab having a surface stained with a plurality of colors to form a selected design and bonded to each colored area a thin filler covering in the form of a composition having substantially the same color as the original stain and including powdered limestone, the several coverings bonding at their respective edges with each other to maintain the color integrity and definition of each area, and the entire covered surface being polished and having the texture of the original slab.

8. A dry, thin limestone slab having one surface stained with a selected color and bonded thereto a thin filler covering in the form of a composition having substantially the same color as the original stain and including powdered limestone, the covered surface being smooth and having the texture of the original slab and the remaining surfaces being coated with paraffin to prevent moisture absorption.

9. The method of coloring a limestone slab consisting in thoroughly drying the slab, staining the slab surface to be exposed with a selected color, bonding to the stained surface a plastic, cementitious powdered limestone composition having substantially the same color as the origi-

nal stain, permitting the composition to dry, applying waterproof varnish to the composition treated surface to smooth the same and provide a glistening surface, and then coating the unstained surfaces of the slab with a waterproof coating to prevent the ingress of moisture.

10. The method of coloring a limestone slab consisting in thoroughly drying the slab, staining the slab surface to be exposed with a selected color, bonding to the stained surface a plastic, 10 cementitious powdered limestone composition having substantially the same color as the original stain, permitting the composition to dry, and then coating the unstained surfaces of the slab with a waterproof coating to prevent the ingress 15 of moisture.

11. A dry, thin limestone slab having one surface stained with a selected color and bonded thereto a thin filler covering in the form of a composition having substantially the same color 20 as the original stain and including powdered limestone, the covered surface being smooth and having the texture of the original slab and the remaining surfaces being covered with a waterproof coating to prevent the ingress of moisture. 25

FREDERICK BLUEM.

KURT BLUEM.